

## UNITED STATES PATENT OFFICE

2,664,399

## COATING AND LUBRICATING COMPOSITION

Arnold F. Kluender, Chicago Heights, Ill., assignor to Mor-Film Company, a corporation of Illinois

No Drawing. Application August 25, 1949,  
Serial No. 112,416

16 Claims. (Cl. 252—18)

1

The present invention relates, generally, to new and useful improvements in coating compositions adapted to be dispersed in water and then applied to the surfaces of metal stock or other metal pieces so as to provide, when dry, an adherent protective film having desirable rustproofing properties, and which also serves as a surface lubricant when the metal stock or piece is worked under pressure.

There is a large number of manufacturers and fabricators who purchase and maintain an inventory of metal stock such as sheets, bars and rods, which they use from time to time in manufacturing and fabricating operations. After being delivered and unloaded, a considerable period of time may elapse before such metal stock is utilized, and during this period the surface of the stock requires protection even though stored under cover. If the metal stock is not protected, it usually has to be cleaned prior to use, and such cleaning is undesirable in that it requires time and adds to costs of production.

According to the present invention, new and improved coating compositions are provided which may easily be dispersed in water and then used for coating such metal stock so as to form upon drying a protective film on the surface of the metal stock. The protective coating or film remains on the metal stock and serves the dual purpose of a lubricating film when the metal stock is subjected to working and drawing operations such as drawing, stamping, shaping, etc. Desirably, the coating compositions may contain one or more addition components in minor amounts which contribute beneficial properties to the protective films, such as substantial rustproofing properties.

The object of my invention, generally stated, is the provision of a composition of matter, usually in dry form, which may readily be dispersed in water so as to provide a composition for coating metal stock which upon drying leaves an adherent film which protects the metal stock during storage and which affords lubrication during working under high pressures.

An important object of the invention is the provision of a new composition which is comparatively inexpensive and easily packaged, stored and handled in granular form which, upon being dispersed in water, provides a coating composition for metal stock such as bar and rod stock, sheet, etc., said coating upon drying providing the stock with an adherent protective film which provides for lubrication when the metal stock is worked under high pressures and stress as in deep drawing operations.

2

Still another object of the invention is the provision of a coating composition in dry granular form, which may readily be dispersed in water and applied to metal stock in that form, so as to provide upon drying a protective film which has lubricating properties in working operations such as deep drawing, said composition also including an ingredient which has rustproofing properties and also lubricating properties.

10 Other objects of the invention will, in part, be obvious and will, in part, appear hereinafter.

For a more complete understanding of the nature and scope of the invention, reference may now be had to the following detailed description thereof wherein certain presently preferred embodiments of the invention are set forth in the examples by way of illustration.

The coating compositions of the present invention consist essentially of 20 to 30 parts by weight of water-soluble, medium titre soap (or the equivalent constituent components) having a titre value of from 22 to 30 and from about 70 to 80 parts by weight of borax. The values of 70 to 80 parts by weight for the borax constituent 20 are based on sodium tetraborate containing 10 molecules of water of crystallization or hydration. If desired, sodium tetraborate which is anhydrous or contains less than 10 molecules of water of hydration may be used, in which case the range of 70 to 80 parts by weight will be correspondingly reduced. For example, when anhydrous sodium tetraborate is used, the range in parts by weight will be from 37 to 42 instead of from 70 to 80.

The preferred embodiments of the invention contain as a third ingredient a small portion of trisodium phosphate, sodium nitrite, or soda ash. These ingredients contribute rustproofing properties to the films coated onto the metal stock, and, in addition, have high temperature lubricating properties when the metal stock is worked as by deep drawing. When such a third ingredient is included in the compositions they will consist essentially of 20 to 30 parts by weight of the water-soluble, medium titre soap, about 65 to 75 parts by weight of the borax and approximately 2 to 5 parts by weight of trisodium phosphate, sodium nitrite, or soda ash. The values of 2 to 5 parts by weight are, as in the case of the borax, based on ingredients containing water of hydration, and when corresponding anhydrous ingredients are employed, these values will be reduced.

In certain embodiments of the invention I may also include from 2 to 5 parts by weight of starch, which improves the properties of the protective films in regard to improved adherence under unusually humid or moist storage conditions.

The formulations set forth in the following examples more fully illustrate the nature of the invention and the preferred methods of practicing it:

## Example 1

|                                  | Parts by weight |
|----------------------------------|-----------------|
| #718 Armour certified flake soap | 25              |
| Borax, granulated                | 70              |
| Tri-sodium phosphate             | 5               |

<sup>1</sup> Medium titre sodium soap of red oil having titre of 28-32° C.

## Example 2

|                                  | Parts by weight |
|----------------------------------|-----------------|
| #718 Armour certified flake soap | 20              |
| Borax, granulated                | 75              |
| Soda ash                         | 5               |

## Example 3

|                                  | Parts by weight |
|----------------------------------|-----------------|
| #718 Armour certified flake soap | 30              |
| Borax, granulated                | 65              |
| Tri-sodium phosphate             | 3               |
| Soda ash                         | 2               |

## Example 4

|                                  | Parts by weight |
|----------------------------------|-----------------|
| #718 Armour certified flake soap | 20              |
| Borax, granulated                | 80              |

## Example 5

|                                  | Parts by weight |
|----------------------------------|-----------------|
| #718 Armour certified flake soap | 30              |
| Borax, granulated                | 70              |

## Example 6

|                                             | Parts by weight |
|---------------------------------------------|-----------------|
| Sodium soap of cottonseed oil (titre 28-32) | 25              |
| Borax, granulated                           | 70              |

## Example 7

|                                               | Parts by weight |
|-----------------------------------------------|-----------------|
| #718 Armour certified flake soap              | 25              |
| Na <sub>2</sub> B <sub>4</sub> O <sub>7</sub> | 33              |
| Sodium nitrite                                | 5               |
| Starch                                        | 5               |

## Example 8

|                                  | Parts by weight |
|----------------------------------|-----------------|
| #718 Armour certified flake soap | 20              |
| Borax, granulated                | 75              |
| Starch                           | 5               |

Medium titre soaps derived from other fatty acids such as corn oil and soya bean oil may also be used in the foregoing formulations to replace all or a part of the medium titre soap of red oil.

Each of the formulations given in the foregoing examples is in the form of a dry granular powder which may be prepared by admixing the ingredients together in the proper proportions. The compositions may be packaged according to standard packaging techniques in known types of packages such as cardboard cartons, barrels or drums.

In use, the dry granular compositions are dispersed or dissolved in water in the ratio of about 1 part by weight of the dry formulation from 5 to 30 parts of water, although this ratio is not critical. Usually the coating solution will be made up in a dip tank or similar receptacle so that the metal stock to be coated may merely be immersed therein and then removed to dry on standing. It will, of course, be understood that the composition can be sprayed or otherwise applied directly to the metal stock.

In the foregoing examples, the medium titre soaps may be in whole, or in part, replaced by the

constituent components in approximately the stoichiometric proportions for forming the soap. That is, instead of using a soap, the coating compositions may be formulated in dry form by admixing the alkali (e. g. caustic soda or caustic potash) and free fatty acid components of the soap in suitable proportions to react and form the soap. From the practical standpoint there may be advantages in using the soap-forming components instead of the soap itself. Thus, there are instances wherein it is cheaper to formulate the soap components of the compositions directly from the alkali and the corresponding free fatty acid, rather than by formulating with the soap itself. Also, a greater degree of flexibility in formulation is possible in formulating with alkali and free fatty acid since there is a much wider range of commercial free fatty acids available for use than the range of suitable medium titre soaps which are commercially available.

The following examples will serve to illustrate embodiments of the invention formulated using alkali and free fatty acid instead of the medium titre soap:

## Example 9

|                      | Parts by weight |
|----------------------|-----------------|
| Caustic soda         | 3.2             |
| Red oil (oleic acid) | 21.8            |
| Borax, granulated    | 70              |
| Tri-sodium phosphate | 5               |

The caustic soda, borax and tri-sodium phosphate are mixed in a suitable mechanical mixer and the red oil may then be sprayed onto the mass and uniformly blended therewith. The caustic soda and red oil will react sufficiently to produce a free-flowing product. The reaction between the alkali and fatty acid will be completed when the product is dissolved in water preparatory to use in coating metal. Heating will hasten the completion of the reaction.

## Example 10

|                      | Parts by weight |
|----------------------|-----------------|
| Caustic soda         | 2.5             |
| Red oil (oleic acid) | 17.5            |
| Borax, granulated    | 75              |
| Soda ash             | 2.5             |
| Starch               | 2.5             |

## Example 11

|                      | Parts by weight |
|----------------------|-----------------|
| Caustic soda         | 3.8             |
| Red oil (oleic acid) | 26.2            |
| Borax, granulated    | 65              |
| Tri-sodium phosphate | 3               |
| Soda ash             | 2               |

## Example 12

|                   | Parts by weight |
|-------------------|-----------------|
| Caustic potash    | 3.3             |
| Oleic acid        | 16.7            |
| Borax, granulated | 75              |
| Sodium nitrite    | 5               |

The fatty acid component in Examples 9-12 may be derived from cottonseed oil, corn oil or soya oil, or other fatty acids which will yield a medium titre soap.

In those formulations made with anhydrous constituents, it may be desirable to add water in an amount sufficient to make up for all or a portion of that normally present as water of crystallization.

It will be apparent that a large number of formulations may be made in view of the fore-

going disclosure, which will vary somewhat with respect to specific percentages and types of ingredients. In all instances, at least about 85% by weight of the formulations will consist together of  $\text{Na}_2\text{B}_4\text{O}_7$ , either hydrated or anhydrous, plus the medium titre soap, either as such or as the corresponding alkali and free fatty acid constituents in approximately stoichiometric proportions. The balance of the formulations, if any, will consist essentially of at least one of the group, trisodium phosphate, sodium nitrite and soda ash, plus starch, if present.

Having fully described my invention and having set forth a number of the preferred embodiments thereof, what is claimed as new is:

1. A new composition of matter adapted to be dispersed in water and used to coat metal stock so as to form upon drying thereon an adherent protective film having rustproofing properties and which serves as a surface lubricant in working the metal stock, and consisting essentially of 20 to 30 parts by weight of a soap material selected from the group consisting of water-soluble medium titre soap having a titre value of from 22 to 30 and the alkali and free fatty acid soap-forming constituents of said soap, 34 to 40 parts by weight of  $\text{Na}_2\text{B}_4\text{O}_7$  calculated on an anhydrous basis, and approximately 2 to 5 parts by weight of at least one member selected from the group consisting of trisodium phosphate, sodium nitrite and soda ash.

2. A new composition of matter adapted to be dispersed in water and used to coat metal stock so as to form upon drying thereon an adherent protective film having rustproofing properties and which serves as a surface lubricant in working the metal stock, and consisting essentially of approximately 20 to 30 parts of a soap material selected from the group consisting of water-soluble medium titre soap having a titre value of from about 22 to 30 and the alkali and free fatty acid soap-forming constituents of said soap, approximately 65 to 75 parts by weight of granulated borax, and approximately 2 to 5 parts by weight of trisodium phosphate.

3. The composition called for in claim 1 wherein said water-soluble medium titre soap is at least one of the group consisting of the sodium and potassium soaps of red oil having a titre within the range of 28-32° C.

4. The composition called for in claim 2 wherein said water-soluble medium titre soap is at least one of the group consisting of the sodium and potassium soaps of red oil having a titre within the range of 28-32° C.

5. The composition called for in claim 1 containing about 2 to 5 parts by weight of starch.

6. The composition called for in claim 2 containing about 2 to 5 parts by weight of starch.

7. A new composition of matter adapted to be dispersed in water and used to coat metal stock so as to form upon drying thereon an adherent protective film which serves as a surface lubricant in working the metal stock, and consisting essentially of from 20 to 30 parts by weight of a soap material selected from the group consisting of 65 water-soluble medium titre soap having a titre value of from 22 to 30 and the alkali and free fatty acid soap-forming constituents of said soap, and from about 37 to 42 parts by weight of  $\text{Na}_2\text{B}_4\text{O}_7$  calculated on an anhydrous basis.

8. The composition called for in claim 7 wherein said water-soluble soap is at least one of the group consisting of the sodium and potassium soaps of red oil having a titre within the range of 28-32° C.

9. A new composition of matter adapted to be dispersed in water and used to coat metal stock so as to form upon drying thereon an adherent protective film which serves as a surface lubricant in working the metal stock, and consisting essentially of from 20 to 30 parts by weight of a soap material selected from the group consisting of water-soluble medium titre soap having a titre value of from 22 to 30 and the alkali and free fatty acid soap-forming constituents of said soap, and from about 70 to 80 parts by weight of granulated borax.

10. The composition called for in claim 7 containing about 2 to 5 parts by weight of starch.

11. The composition called for in claim 8 containing about 2 to 5 parts by weight of starch.

12. A new composition of matter adapted to be dispersed in water and used to coat metal stock so as to form upon drying thereon an adherent protective film having rustproofing properties and which serves as a surface lubricant in working the metal stock, and consisting essentially of at least about 85% by weight of a mixture of 20 to 30 parts by weight of a soap material selected from the group consisting of (1) water-soluble medium titre soap having a titre value of from 22 to 30 and (2) the alkali and free fatty acid soap-forming constituents of said soap, and 70 to 80 parts by weight of borax.

13. A new composition of matter adapted to be dispersed in water and used to coat metal stock so as to form upon drying thereon an adherent protective film having rustproofing properties and which serves as a surface lubricant in working the metal stock, and consisting essentially of approximately 25 parts by weight of the sodium soap of red oil having a titre within the range of 28-32° C., approximately 70 parts by weight of granulated borax, and approximately 5 parts by weight of trisodium phosphate.

14. The composition of claim 13 wherein the soap is replaced by caustic soda and red oil in soap-forming proportions.

15. The composition of claim 12 wherein said soap is at least in part replaced by its alkali and free fatty acid constituents.

16. A new composition of matter adapted to be dispersed in water and used to coat metal stock so as to form upon drying thereon an adherent protective film which serves as a surface lubricant in working the metal stock, and consisting essentially of approximately 3.2 parts by weight of caustic soda, approximately 21.8 parts by weight of red oil, approximately 70 parts by weight of borax and approximately 5 parts by weight of trisodium phosphate.

ARNOLD F. KLUENDER.

References Cited in the file of this patent

UNITED STATES PATENTS

| Number     | Name     | Date          |
|------------|----------|---------------|
| Re. 23,184 | Whitbeck | Dec. 20, 1949 |
| 2,074,224  | Johnson  | Mar. 16, 1937 |
| 2,252,385  | Orozco   | Aug. 12, 1941 |
| 2,469,473  | Orozco   | May 10, 1949  |
| 2,530,837  | Orozco   | Nov. 21, 1950 |